

1

2,941,005

**1,2-DIAMINO-1-ALKENE COMPOUNDS**

John E. Mahan, Bartlesville, Okla., assignor to Phillips Petroleum Company, a corporation of Delaware

No Drawing. Filed July 29, 1955, Ser. No. 525,347

4 Claims. (Cl. 260—583)

This invention relates to fast burning fuels. In one aspect this invention relates to rocket fuels. In another aspect this invention relates to hypergolic fuels. In another aspect this invention relates to a method for propelling rockets. In another aspect this invention relates to 1,2-diamino-1-alkenes as new compounds. In still another aspect this invention relates to new fuel compositions comprising a liquid hydrocarbon and at least one of said 1,2-diamino-1-alkenes.

This application is a continuation-in-part of my pending application Serial No. 366,381, filed July 6, 1953 which in turn is a continuation-in-part of my pending application Serial No. 257,973, filed November 23, 1951, now abandoned.

My invention is concerned with new and novel rocket propellants and their utilization. A rocket or jet propulsion device, such as is discussed herein is defined as a rigid container for matter and energy, so arranged that a portion of the matter can absorb the energy in kinetic form and subsequently eject it in a specified direction. The type rocket to which my invention is particularly applied is that type rocket propulsion device designated as a "pure" rocket, i.e., a thrust producer which does not make use of its surrounding atmosphere. A rocket of the type with which my invention is concerned is propelled in response to the steps of introducing a propellant material into a combustion chamber therein, and burning it under conditions that will cause it to release energy at a high but controllable rate immediately after its entry into the combustion chamber.

Rocket propellants in liquid form are advantageously utilized inasmuch as the liquid propellant materials can be carried in a light weight, low pressure vessel and thereafter be pumped into the combustion chamber. It is thus necessary that the combustion chamber, although being strong enough to stand high pressure and temperature, need be only large enough to insure combustion. The flow of liquid propellants into the combustion chamber can be regulated at will so that the thrust resulting from continuous or intermittent bursts of power can be sustained. Intermittent burning of the fuel contributes to a longer life of the combustion chamber and of the thrust nozzle.

Various methods and liquid combinations have been found to be useful as rocket propellants. Some propellants consist of a single material, and are termed "monopropellants." Those propellants involving two materials are termed "bipropellants" and normally consist of an

2

oxidizer and a fuel. Hydrogen peroxide and nitromethane are each well known monopropellants. Well known bipropellants include hydrogen peroxide or liquid oxygen as the oxidant with a fuel component such as ethyl alcohol-water, ammonia, hydrazine or hydrogen. Additional known bipropellants include nitric acid as the oxidizer with aniline or furfural alcohol as the hypergolic fuel component.

When employing 90-100 percent nitric acid, i.e., "white fuming nitric acid" as the oxidizer in a rocket bipropellant fuel, it is often necessary, dependent upon the specific fuel component, to obtain more effective ignition than would normally be obtained, by dissolving from 6 to 23 percent by weight of nitrogen dioxide in white fuming nitric acid, thereby forming "red fuming" nitric acid. A fuel component of the bipropellant type described herein is spontaneously ignited upon contacting the oxidizer. For this reason such a bipropellant material is referred to herein as being "hypergolic." A ratio of oxidizer to 20 hypergolic fuel, based upon stoichiometric amounts, can be utilized within the limits of 0.5:1 to 1.5:1 if desired. The efficiency of combustion is less at a ratio below 1:1 and the use of the oxidizer is less economical at ratios above 1:1. However, practical consideration may necessitate the use of higher ratios, even as high as 6:1.

Each of the following objects of the invention will be obtained by the various aspects of this invention.

An object of this invention is to provide new rocket propellants. Another object of the invention is to provide a novel hypergolic fuel. Another object of the invention is to provide a method for producing immediate thrust to a rocket-type device. Another object is to provide as new compounds the 1,2-diamino-1-alkenes characterized by the structural formula given and defined below. Another object is to provide an improved fast-burning fuel. Other and further objects will be apparent to those skilled in the art upon study of the accompanying disclosure.

In accordance with the broad aspects of this invention, I have found that organic polyamines, either in the presence or absence of normally liquid hydrocarbons form a fuel component which is highly "hypergolic" and suitable for use in the propulsion of rockets, guided missiles, and the like, in conjunction with an oxidizer. I have further found that these organic polyamines together with selected mercaptans, both more fully set forth hereinbelow, either in the presence or absence of normally liquid hydrocarbons, form a fuel component which is also highly "hypergolic" and suitable for the uses set forth above. The fuels of the present invention are composed of (1) at least one organic polyamine or mixture thereof, or (2) at least one organic polyamine or mixture thereof with at least one selected mercaptan, either of the latter components being suitable in a major or minor amount. When a selected mercaptan is used as one of the fuel constituents, it is preferred that the mixtures contain at least 10 percent of the organic polyamines and not more than 90 percent of the organic polyamines. In some instances, lesser amounts of the organic polyamine substituents can be used.

In accordance with the invention in my copending ap-

lication Serial No. 257,973, filed November 23, 1951, there are disclosed and now being claimed those organic polyamines selected from the group consisting of 1,3-butanediamine, 1,2-propanediamine, triethylenetetramine, and tetraethylenepentamine.

In accordance with the invention in my copending application Serial No. 366,381, filed July 6, 1953 there are disclosed and now being claimed those organic polyamines which contain at least two



groups attached to one or more carbon atoms, wherein R is selected from the group consisting of a hydrogen atom and hydrocarbon radicals selected from the group consisting of alkyl, alkenyl, cycloalkyl, cycloalkenyl, aryl, alkaryl, and aralkyl radicals and the hydrocarbon of said polyamine is selected from the same group, the total number of carbon atoms in said polyamine being not greater than 30 and at least one R of at least two



groups being a hydrocarbon radical.

In both of the said copending applications the carbon atom to which the substituent



group is attached may be a cyclic (carbocyclic) carbon atom, a carbon atom of a side chain group attached to a cyclic (carbocyclic) carbon atom or a carbon atom of an acyclic molecule.

The following organic polyamines are useful in the practice of the invention of my copending application Serial No. 366,381: the aliphatic polyamines which include the various alkane polyamines such as

N,N'-diethyl-1,4-hexanediamine;  
N,N,N',N'-tetraallylmethylenediamine;  
N,N,N',N'-tetramethylmethylenediamine;  
N,N,N',N'-tetramethylmethylethane-1,2-diamine;  
N,N,N',N'-tetramethylbutane-1,4-diamine;  
N,N,N',N'-tetramethylpropane-1,3-diamine; and  
N,N,N',N'-tetramethylpropane-1,2-diamine.

Various alkenylene polyamines are also very efficient hypergolic materials and include

N,N,N',N'-tetramethylpropene-1,3-diamine;  
N,N,N',N'-tetraallylpropene-1,3-diamine;  
N,N,N',N'-tetraethylpropene-1,3-diamine;  
N,N,N',N'-tetra(2-methylallyl)propene-1,3-diamine;  
N,N,N',N'-tetracrotylpropene-1,3-diamine;  
N,N'-diallyl-N,N'-di(3-butene)propene-1,3-diamine;  
N,N,N',N'-tetraallyl-2-methylpropene-1,3-diamine;  
N,N'-diallyl-N,N'-dimethylpropene-1,3-diamine;  
N,N'-dicyrtoyl-N,N'-dipropylpropene-1,3-diamine;  
N,N,N',N'-tetramethyl-2-methylpropene-1,3-diamine; and the like.

In addition to the above recited specific compounds, the total reaction mixture or fractions thereof from the preparation of N,N,N',N'-tetraallyl-, tetramethylallyl-, or tetracrotylpropene-1,3-diamine, is useful as constituent of hypergolic fuel compositions according to the said Serial No. 366,381. These compounds are known in the art and can be prepared by the manner described in U.S. Patent 2,565,529 by C. W. Smith, wherein a suitable alpha, beta-unsaturated aldehyde is reacted with one or more secondary monoamines having attached to the nitrogen atom at least one alkenyl group with an olefinic bond in the 2,3-position relative to the hydrogen atom or by other similar methods.

As indicated hereinbefore, and in accordance with my invention, the amino groups of the above-described polyamines may be substituted amino groups containing the above-named hydrocarbyl groups or other substituent

groups containing only carbon, hydrogen and nitrogen atoms.

Further according to the invention there are now provided as new compounds the 1,2-diamino-1-alkenes characterized by the structural formula



10 wherein: R, is a member selected from the group consisting of a hydrogen atom, alkyl, cycloalkyl, alkenyl, and cycloalkenyl hydrocarbon radicals; each R is a member selected from the group consisting of alkyl, cycloalkyl, alkenyl and cycloalkenyl hydrocarbon radicals, and the 15 R's can be alike and unlike; the total number of carbon atoms in the molecule does not exceed 24; and the total number of carbon atoms in R<sub>1</sub> does not exceed 8. It is to be understood that herein and in the claims the above 20 named hydrocarbon radicals includes the various combinations of said radicals such as alkylcycloalkyl, cycloalkenylalkyl, cycloalkylalkenyl, alkylcycloalkenyl, alkenylcycloalkenyl, etc.

Included in the group of new compounds represented by the above formula are,

N,N,N',N'-tetramethyl-1,2-diaminoethylene,  
N,N,N',N'-tetraethyl-1,2-diaminoethylene,  
N,N,N',N'-tetramethyl-1,2-diamino-1-butene,  
N,N,N',N'-tetramethyl-1,2-diamino-1-hexene,  
N,N'-dimethyl-N,N'-diethyl-1,2-diaminoethylene,  
N,N-dimethyl-N,N'-diethyl-1,2-diaminoethylene,  
N,N-diethyl-N,N'-diallyl-1,2-diaminoethylene,  
N,N,N',N'-tetrapropyl-1,2-diamino-1-decene,  
N,N'-dicyclohexyl-N,N'-dimethyl-1,2-diaminoethylene,  
N,N,N',N'-tetrapropyl-1,2-diamino-4-cyclohexyl-1-butene,  
N,N,N',N'-tetraethyl-2-cyclohexyl-1,2-diaminoethylene,  
N,N,N',N'-tetramethyl-1,2-diamino-3,7-dimethyl-1,7-octadiene,  
N,N,N',N'-tetrabutyl-2-ethylcyclohexyl-1,2-diaminoethylene, and  
40 N,N'-dimethyl-N,N'-di-t-hexyl-4-cyclopentenyl-1,2-diamino-1-butene,  
N,N'-dimethyl-N,N'-di(2-butene)-5-cyclopentyl-1,2-diamino-1,4-pentadiene,  
N,N'-dimethyl-N,N'-di(2-cyclopentylethyl)-1,2-diamino-4-methyl-1-pentene,  
N,N'-diethyl-N,N'-di(3-ethyl-2-cyclopentenyl)1,2-diamino-1-propene,  
N,N'-dimethyl-N,N'-di(5-allyl-2-cyclohexenyl)1,2-diaminoethylene.

50 I have further found that the new compounds of my invention are especially useful as hypergolic fuels. Indeed, said new compounds are superior to any previously known hypergols as shown by the data given below in Example XIV and Table II. Examples I to XII, given 55 below, are included for comparison purposes to show the superiority of my new compounds as hypergolic fuels as compared with other organic polyamines.

The new compounds of my invention can be prepared by reacting under suitable conditions, an alpha-halo-aldehyde, having at least one hydrogen atom attached to the carbon atom alpha to the aldehyde group, with a secondary amine as disclosed and claimed in the copending application of R. C. Doss and H. W. Bost, Serial No. 525,346, filed July 29, 1955, now Patent No. 2,881,217, issued April 7, 1959. Said method of preparing my new compounds is illustrated below in Example XIII and Table I.

Representative halo-aldehyde which can be used in preparing my new compounds include, among others, the following: chloroacetaldehyde, 2-bromo-propionaldehyde, 2-chloro-n-butylaldehyde, 2-chloro-3,3-dimethyl-1-butylaldehyde, 2-chlorocapraldehyde, fluoroacetaldehyde, 2-iodopropionaldehyde, 2-chloro-4-cyclohexylbutyraldehyde, 2-chloro-2-cyclohexyl-acetaldehyde, and 2-chlorocitronellaldehyde.

Representative secondary amines which can be used in preparing my new compounds include, among others, the following: dimethylamine, diethylamine, methylethylamine, dibutylamine, dipropylamine, diisopropylamine, diallylamine, and N-methylcyclohexylamine.

The fuel constituents of the present invention are hypergolic in an undiluted state and are also hypergolic when admixed with non-hypergolic materials, particularly hydrocarbons, in a state of dilution as high as 70 percent by volume of diluent when white fuming nitric acid is used as the oxidant. Suitable non-hypergolic materials which also may form a portion of the fuel composition include paraffin, cycloparaffin, and aromatic hydrocarbons in the C<sub>5</sub> to C<sub>30</sub> range or mixtures thereof, preferably the normally liquid materials. Examples of such hydrocarbon fuels are normal pentane, normal hexane, normal heptane, benzene, kerosene, iso-octane, diisopropyl, diisobutylene, cyclohexene, cyclohexane, isodecane, methylcyclohexane, toluene, hexadecane, eicosane, hexacosane, pentatricontane, picene, cyclononacosane, methylal tetraphenylethylene and the like. Hydrocarbons in the C<sub>5</sub> to C<sub>18</sub> range are preferred.

Other oxidizers are suitable oxidants for these hypergolic fuels in addition to white or red fuming nitric acid and can be used in the bipropellant fuel compositions of our invention. Suitable oxidants include materials such as hydrogen peroxide, ozone, nitrogen tetroxide, liquid oxygen and mixed acids, especially anhydrous mixtures of nitric and sulfuric acids such as 80 to 90 percent by volume of white or red fuming nitric acid and 10 to 20 percent by volume anhydrous or fuming sulfuric acid. It is within the scope of this invention to employ, preferably dissolved in the oxidizer, ignition catalysts or oxidation catalysts. These oxidation catalysts include certain metal salts, such as the chlorides and naphthenates of iron, zinc, cobalt and similar heavy materials.

As an added feature of this invention my new compounds are also useful for providing fast burning fuels for use in rocket engines and the like wherein a hypergolic fuel is not necessarily required. For example, the fuel components of this invention are dispersed in a hydrocarbon, such as the hydrocarbon diluents described above. Even if the resulting solution is not hypergolic with an oxidant such as fuming nitric acid, it can be used together with an oxidant and a suitable igniter as a rocket propellant. These fast burning fuels are particularly useful if, for various reasons, a hypergolic fuel is not desired or required. The organic polyamines of this invention may be added to a hydrocarbon fuel in a minor amount, usually from 1 to 20 percent by volume of the total mixture to produce fast-burning fuels which are non-hypergolic. Suitable fast-burning fuels comprise from 1 to 20 percent by volume of an organic polyamine described above with 90 to 99 percent by volume of a petroleum fraction gasoline boiling range. Specifically, such a fuel can comprise between 1 and 20 percent by volume of a 1,2-diamino-1-alkene and 80 to 99 percent by volume normal heptane.

As pointed out above, selected mercaptans can be used to form a portion of the hypergolic fuel constituents of this invention in admixture with the above described organic polyamines. Likewise selected mercaptans can be used with my new 1,2-diamino-1-alkenes. The mercaptans which are suitable for use as such a hypergolic fuel constituent include compounds of the general formula RSH, wherein R is selected from the group consisting of alkyl and alkenyl groups containing from 3 to 10 carbon atoms. Illustrative of the mercaptans used in this invention are tert-butyl mercaptan, isopropyl mercaptan, allyl mercaptan, n-butyl mercaptan, n-hexyl mercaptan, tert-hexyl mercaptan, tert-octyl mercaptan, nonyl mercaptan, tert-decyl mercaptan, 2-butene-1-thiol, 3-butene-1-thiol, isobutyl mercaptan, and the like.

A fuel of the present invention, i.e., mixtures consisting of at least one 1,2-diamino-1-alkene and at least one mercaptan are hypergolic in an undiluted state and are

also hypergolic when admixed with non-hypergolic materials, particularly those normally liquid hydrocarbons set forth above, when using such hydrocarbons in amounts as high as 50 percent by volume of hydrocarbon when white fuming nitric acid is used as the oxidant.

The invention is further illustrated in the following examples. The reactants and their proportions and the specific ingredients are presented as being typical and not to be construed as unduly limiting the invention.

#### EXAMPLE I

The materials described below were tested for spontaneous ignition employing fuming nitric acids as the oxidizer. In each test one part by volume of a hydrocarbon polyamine solution was dropped into a vessel containing 2.3 parts by volume fuming nitric acid. The candidate polyamine was dissolved in n-heptane or benzene so as to determine the maximum hydrocarbon dilution possible while still retaining the property of hypergolicity. Those mixtures below the maximum percentage were all hypergolic, including the undiluted polyamine itself. Tests were conducted at room temperature, about 70° F. The results are set forth below.

| Polyamine              | Oxidant                  | Maximum Dilution, Percent volume n-heptane or benzene |
|------------------------|--------------------------|-------------------------------------------------------|
| 1,3-butanediamine      | Red Fuming Nitric Acid   | 1 60                                                  |
| Do                     | White Fuming Nitric Acid | 1 40                                                  |
| triethylenetetramine   | Red Fuming Nitric Acid   | 2 50                                                  |
| tetraethylenepentamine | do                       | 2 45                                                  |

<sup>1</sup> n-Heptane diluent.

<sup>2</sup> Benzene diluent.

#### EXAMPLE II

A reaction flask fitted with thermometer, dropping funnel, reflux condenser and stirring unit was charged with a mixture of 50 grams of finely powdered anhydrous potassium carbonate, 150 grams of diethyl ether and 194 grams of diallylamine. As the mixture was stirred vigorously, 56 grams of acrolein were slowly added with cooling to maintain the reaction mixture between 10 and 15° C. (50 to 59° F.). After all the acrolein had been added, the reaction mixture was kept at 5 to 10° C. (41 to 50° F.) and stirred for 17 hours. The contents of the reactor were then filtered to remove the solid desiccant; a dark-red filtrate was recovered. The ether and low boiling components, including unreacted acrolein and diallylamine, were removed by fractional distillation. The higher boiling material was then transferred to a vacuum distillation apparatus and distilled under reduced pressure. A summary of the distillation results is presented in the following table:

| Fraction                                       | Head Temperature, °C. | Kettle Pressure, mm. | Refractive Index at 20° C. | Wt., Grams | Wt. Percent |
|------------------------------------------------|-----------------------|----------------------|----------------------------|------------|-------------|
| No. 1, Light Materials                         | <93                   | <1                   | -----                      | 97.8       | 29.2        |
| No. 2, N,N,N',N'-tetraallylpropene-1,3-diamine | 93-105                | <1.5                 | 1.4053                     | 57.2       | 17.1        |
| No. 3, Unidentified heavier materials          | 135-200               | >8                   | 1.5182                     | 27.9       | 8.3         |
| Residue                                        | >200                  | -----                | -----                      | 152.0      | 45.4        |
| Total                                          | -----                 | -----                | -----                      | 334.9      | 100         |

#### EXAMPLE III

N,N,N',N'-tetraallylpropene-1,3-diamine and the other materials recovered from the fractionation of Example I were tested for spontaneous ignition employing fuming nitric acid as the oxidant. The temperature of the fuel and oxidant was maintained at room temperature (21° C.). In each test 0.13 ml. of the fuel or a diluted solution thereof was dropped into a 1" x 8" test tube con-

taining 0.3 ml. of fuming nitric acid. The inert diluent (n-heptane) was employed to determine the amount of dilution which each fuel would tolerate and retain its hypergolic properties. The results are set forth in the following table.

| Fuel                                                      | Oxidant        | Maximum Percent Dilution with n-heptane with Retention of Hypergolicity |
|-----------------------------------------------------------|----------------|-------------------------------------------------------------------------|
| Fraction No. 1                                            | {RFNA<br>WFNA} | 50                                                                      |
| Fraction No. 2 (N,N,N',N'-tetraallylpropene-1,3-diamine). | {RFNA<br>WFNA} | 70                                                                      |
| Fraction No. 3                                            | {RFNA<br>WFNA} | 60                                                                      |

In addition to the room temperature tests previously described, N,N,N',N'-tetraallyl-1,3-diaminopropene and other materials recovered from the fractionation procedure of Example I were also tested for spontaneous ignition at  $-40^{\circ}\text{C}$ . Prior to testing, the temperature of the fuel and oxidant was lowered to  $-40^{\circ}\text{C}$ . Tests were conducted employing 0.13 ml. of fuel or a diluted solution thereof and 0.3 ml. of fuming nitric acid. Results are recorded below.

| Fuel                                                      | Oxidant        | Maximum Percent Dilution with n-heptane with Retention of Hypergolicity at $-40^{\circ}\text{C}$ . |
|-----------------------------------------------------------|----------------|----------------------------------------------------------------------------------------------------|
| Fraction No. 2 (N,N,N',N'-tetraallylpropene-1,3-diamine). | {RFNA<br>WFNA} | 30                                                                                                 |
| Fraction No. 3                                            | {WFNA}         | 10                                                                                                 |

In addition to the above tests, the crude reaction mixture obtained from the procedure of Example I was also tested for self-ignition properties. Prior to testing, ether and other low boiling materials were removed by heating the reaction mixture in a warm water bath under reduced pressure provided by a water aspirator. Results are recorded below.

| Fuel                                                                                                  | Oxidant        | Maximum Percent Dilution with n-heptane with Retention of Hypergolicity |
|-------------------------------------------------------------------------------------------------------|----------------|-------------------------------------------------------------------------|
| Crude Reaction Mixture from the Run Described in Example I (Ether and low boiling materials removed). | {RFNA<br>WFNA} | Not diluted.                                                            |
| Do.                                                                                                   | {RFNA<br>WFNA} | 60.                                                                     |

#### EXAMPLE IV

A run for the preparation of N,N,N',N'-tetraallylpropene-1,3-diamine was conducted in the manner described in Example I except that the reaction mixture was stirred for 12.5 hours. The reaction mixture was very dark in color and viscous. This material was distilled to remove unreacted diallylamine and other volatile materials leaving a black, plastic residue in the kettle. This material was tested for spontaneous ignition employing fuming nitric acid as oxidant. Tests were conducted with the fuel and oxidant maintained at room temperature ( $21^{\circ}\text{C}$ ). In the first test, a small particle of the solid, plastic residue was dropped into 0.3 ml. of fuming nitric acid in a  $1'' \times 8''$  test tube. In addition this residue was dissolved in n-heptane and the maximum dilution that the material would tolerate and maintain its self-ignition properties was determined. 0.13 ml. of fuel solution was employed with 0.3 ml. of fuming nitric acid as described in the test procedure of Example IV. Results are set forth below.

| 5                                      | Fuel            | Oxidant        | Maximum Percent Dilution with n-heptane with Retention of Hypergolicity |
|----------------------------------------|-----------------|----------------|-------------------------------------------------------------------------|
| 10                                     | Plastic residue | {RFNA<br>WFNA} | Not diluted.                                                            |
| Plastic residue dissolved in n-heptane | {RFNA<br>WFNA}  | 50.<br>50.     | Do.<br>Do.                                                              |

#### EXAMPLE V

A run for the preparation of N,N,N',N'-tetraallylpropene-1,3-diamine was conducted in the manner described in Example I except that the reaction mixture was stirred for 16 hours. After filtering off the potassium carbonate, the reaction mixture was stripped of ether. Then half of the de-etherified material was refluxed to remove everything up to diallylamine under reduced pressure (head temperature  $35^{\circ}\text{C}$ , corr.). The remaining half of this material was refluxed to remove everything up to and including diallylamine under reduced pressure (head temperature,  $117^{\circ}\text{C}$ , corr.). These two materials were tested for self-ignition properties at  $21^{\circ}\text{C}$ . and at  $-40^{\circ}\text{C}$ . in the manner set forth in previous examples. Results are recorded below:

| 30                                              | Fuel | Test Temperature, $^{\circ}\text{C}$ . | Oxidant        | Maximum Dilution with n-heptane with Retention of Hypergolicity |
|-------------------------------------------------|------|----------------------------------------|----------------|-----------------------------------------------------------------|
| Crude product (ether removed).                  |      | 21                                     | {RFNA<br>WFNA} | 70                                                              |
| Do.                                             |      | -40                                    | {RFNA<br>WFNA} | 20                                                              |
| Crude product (ether and diallylamine removed). |      | 21                                     | {RFNA<br>WFNA} | 70                                                              |
| Do.                                             |      | -40                                    | {RFNA<br>WFNA} | 40                                                              |

#### EXAMPLE VI

A drop test apparatus comprising an injection nozzle inserted to within  $1''$  of the bottom of a  $1'' \times 8''$  test tube was employed to determine the ignition delay in milliseconds of N,N,N',N'-tetraallylpropene-1,3-diamine. A small quantity of fuel (0.2 ml.) was placed in the bottom of the test tube and 0.3 ml. of white fuming nitric acid was injected into the fuel. A constant pressure nitrogen surge chamber provided a source of approximately 40 p.s.i.g. pressure to inject the oxidizer into the fuel. A solenoid coil actuated the injector to provide an accurately metered amount of oxidant. The ignition delay interval was determined as the time between contact of the oxidizer with the fuel and the presence of flame as sensed by a photocell.

N,N,N',N'-tetraallylpropene-1,3-diamine was tested employing the apparatus described and was found to have an average ignition delay of 6.3 milliseconds.

This is an extremely short delay compared to known hypergolic fuels, for example, furfuryl alcohol, a known hypergolic fuel, had an ignition delay of 27 milliseconds as determined by the same apparatus and test procedure.

#### EXAMPLE VII

N,N,N',N'-Tetramethylpropene-1,3-diamine was prepared from dimethylamine and acrolein by substantially the same procedure as previously employed for N,N,N',N'-tetraallylpropene-1,3-diamine. The crude material, in 73.8 percent yield, was distilled in an 18-inch column. A 30 percent theoretical yield of distilled product was obtained, along with 22 percent solid kettle residue.

These materials were examined for dilution data and ignition delay with the drop tester using standard techniques.

| Material                                        | B.P.,<br>°C. | $n_{D^{20}}$ | Toluene Dilution |      |         |       | Ignition Delay,<br>milliseconds |  |
|-------------------------------------------------|--------------|--------------|------------------|------|---------|-------|---------------------------------|--|
|                                                 |              |              | Room temp.       |      | -40° C. |       |                                 |  |
|                                                 |              |              | RFNA             | WFNA | RFNA    | WFNA  |                                 |  |
| N,N,N',N'-Tetramethylpropene-1,3-diamine.       | 148          | 1.4589       | 70               | 70   | 10      | 10    | 15.5 @ 24° C.                   |  |
| Crude N,N,N',N'-Tetramethylpropene-1,3-diamine. | -----        | 1.4668       | 70               | 70   | 20      | 20    | 10.5 @ 24° C.                   |  |
| Plastic kettle product.                         | -----        | -----        | Hypergolic       |      | -----   | ----- | -----                           |  |

<sup>1</sup> At 10.3 mm. Hg.

### EXAMPLE VIII

Each of the fuel mixtures described hereinbelow was tested for spontaneous ignition employing fuming nitric

manner described hereinbefore. Tests were conducted with fuel and oxidant at room temperature (21° C.). Results are recorded below.

| Fuel Composition                                                                    | Oxidant                                              | Maximum Percent Dilution with n-Heptane with Retention of Hypergolicity |
|-------------------------------------------------------------------------------------|------------------------------------------------------|-------------------------------------------------------------------------|
| 100 percent tert-butyl mercaptan.                                                   | (Red Fuming Nitric Acid<br>White Fuming Nitric Acid) | No ignition.<br>Do.                                                     |
| 5 weight percent of the residue described above, dissolved in tert-butyl mercaptan. | (Red Fuming Nitric Acid<br>White Fuming Nitric Acid) | 40.<br>50.                                                              |

acid as the oxidant. The temperature of the fuel and oxidant was maintained at 21° C. In each test, 0.13 ml. of the fuel or a diluted solution thereof was dropped into a 1 inch by 8 inch test tube containing 0.3 ml. of fuming nitric acid. The inert diluent was employed to determine the amount of dilution which each fuel would tolerate and retain its hypergolic properties. The results are set forth below.

30

### EXAMPLE X

A run for the preparation of N,N,N',N'-tetraallylpropene-1,3-diamine was conducted in the manner described in Example III except that the reaction mixture was stirred for 16 hours. After filtering off the potassium carbonate the reaction mixture was stripped of ether. A portion of this material was fractionated to remove

| Fuel Composition                                                                                | Oxidant                                              | Maximum Percent Dilution with n-Heptane with Retention of Hypergolicity |
|-------------------------------------------------------------------------------------------------|------------------------------------------------------|-------------------------------------------------------------------------|
| 100% tert-butyl Mercaptan.                                                                      | (Red Fuming Nitric Acid<br>White Fuming Nitric Acid) | No ignition.<br>Do.                                                     |
| 10 volume percent N,N,N',N'-tetraallylpropene-1,3-diamine <sup>1</sup> in tert-butyl mercaptan. | (Red Fuming Nitric Acid<br>White Fuming Nitric Acid) | 20.<br>10.                                                              |

<sup>1</sup> Prepared by the run described in Example III.

### EXAMPLE IX

A run for the preparation of N,N,N',N'-tetraallylpropene-1,3-diamine was conducted in the manner described in Example III except that the reaction mixture was stirred for 12.5 hours. The reaction mixture was

55

everything up to and including diallylamine under reduced pressure (head temperature 117° C., corr.). This material was admixed with tert-butyl mercaptan in varying proportions and the fuel compositions so formed were tested for self-ignition properties by the process described in previous examples. Results are set forth below.

| Fuel Composition                                                                           | Oxidant                                              | Maximum Percent Dilution with n-Heptane with Retention of Hypergolicity |
|--------------------------------------------------------------------------------------------|------------------------------------------------------|-------------------------------------------------------------------------|
| 100 percent tert-butyl mercaptan.                                                          | (Red Fuming Nitric Acid<br>White Fuming Nitric Acid) | No ignition.<br>Do.                                                     |
| 10 percent crude N,N,N',N'-tetraallyl-1,3-diaminopropene (ether and diallylamine removed). | (Red Fuming Nitric Acid<br>White Fuming Nitric Acid) | 20.<br>20.                                                              |

very dark in color and viscous. This material was distilled to remove unreacted diallylamine and other volatile materials, leaving a black, plastic residue in the kettle. A small amount of this residue was dissolved in tert-butyl mercaptan (readily soluble) and the composition so formed was tested for self-ignition properties in the

70

### EXAMPLE XI

Several of the alkane polyamines and alkenylene polyamines were tested for ignition delays with a drop tester, injecting while fuming nitric acid into a small quantity of fuel and determining the ignition delay interval between the contact of the acid and fuel and the presence of flame

75

as sensed by a photocell. The materials and ignition delays are set forth below.

| Material                                 | Ignition Delay with White Fuming Nitric Acid, Milliseconds at 75° F. |
|------------------------------------------|----------------------------------------------------------------------|
| N,N,N',N'-tetramethylmethylenediamine    | 95                                                                   |
| N,N,N',N'-Tetramethylpropane-1,3-diamine | 9                                                                    |
| N,N,N',N'-Tetramethylpropane-1,2-diamine | 6                                                                    |

## EXAMPLE XII

Several additional alkane polyamines and alkenylene polyamines were tested for ignition delays with a drop tester, injecting white or red fuming nitric acid into a small quantity of fuel and determining the ignition delay interval between the contact of the acid and fuel and the presence of flame, as sensed by a photocell. The materials and ignition delays are set forth below.

| Material                                   | Ignition Delay, Milliseconds, at 75° F. |                          |
|--------------------------------------------|-----------------------------------------|--------------------------|
|                                            | Red Fuming Nitric Acid                  | White Fuming Nitric Acid |
| N,N,N',N'-tetramethylmethane-1,2-diamine   | 9.3                                     | 12                       |
| N,N,N',N'-Tetramethylbutane-1,2-diamine    | 14                                      | 16                       |
| N,N,N',N'-Tetramethyl-1-butene-3,4-diamine | 4.1                                     | 4.6                      |
| N,N,N',N'-2-Pentamethylpropane-1,3-diamine | 22                                      | 24                       |
| N,N,N',N'-Tetramethylbutane-1,4-diamine    | 7.4                                     | 7.4                      |
| N,N,N',N'-Tetramethyl-2-butene-1,4-diamine | 4.3                                     | 4.3                      |
| N,N,N',N'-Tetramethylhexane-1,6-diamine    | 8.8                                     | 5.3                      |

## EXAMPLE XIII

To a one liter glass reaction vessel there was added 200 milliliters of methylcyclopentane and 220 milliliters of dimethylamine. The reaction vessel was placed in an acetone-Dry Ice bath and, after cooling to -8° C., 186 grams of a 40 percent aqueous solution of chloroacetaldehyde was added dropwise with stirring. The temperature of the reaction mixture was maintained between -10 and 0° C. for the approximately 30 minutes required to add the chloroacetaldehyde. The temperature of the black colored mixture was permitted to rise to room temperature (about 25° C.) and stirred 2 hours at this temperature.

The aqueous layer of the reaction mixture was separated and extracted 3 times with methylcyclopentane. The extracts were then combined with the non-aqueous phase of the reaction mixture, dried overnight with magnesium sulfate, filtered and distilled at reduced pressure. The distillation data is given in Table I with the product indicated in Cuts 3 to 7 inclusive. It is presently believed that the reaction can be represented by the equation



A sodium fusion was made on Cut Number 5 and a qualitative test for halogen indicated none was present. Solutions of potassium permanganate and bromine were absorbed by the product, indicating the presence of a double bond. A titration of a portion of the product, made with hydrochloric acid, caused decomposition yielding the free amine.

Cuts 4 and 7 were hydrogenated in the presence of nickel in a Parr hydrogenation bomb at 40 p.s.i.g. and room temperature. The refractive index of the hydrogenated sample was 1.4180 at 25° C. as compared with 1.4170 at 25° C. for a sample of N,N,N',N'-tetramethylmethylenediamine. These tests served to characterize the product as N,N,N',N'-tetramethyl-1,2-diaminoethylene.

Table I  
[Pressure—15 mm. mercury.]

| 5 | Cut No. | Overhead Temp., ° C. | Distillate Collected, gms. | Distillate, Refractive Index |
|---|---------|----------------------|----------------------------|------------------------------|
| 1 |         |                      | 38.4                       |                              |
| 2 |         | 30                   | 62.8                       | 1.4207                       |
| 3 |         | 33                   | 9.1                        | 1.4643                       |
| 4 |         | 38                   | 9.8                        | 1.4655                       |
| 5 |         | 40                   | 9.0                        | 1.4658                       |
| 6 |         | 40                   | 8.4                        | 1.4658                       |
| 7 |         | 40                   | 4.8                        | 1.4648                       |

|    |            |       |
|----|------------|-------|
| 15 | Charge     | Grams |
|    | Residue    | 20.1  |
|    | Trap       | 170.0 |
|    | Distillate | 142.3 |
|    | Loss       | 4.1   |

<sup>1</sup> Mainly methylcyclopentane—collected in a trap maintained in a Dry Ice-acetone bath to prevent vapors from entering vacuum pump.

20 The product yield was 38 percent of theoretical based on the chloroacetaldehyde charged.

## EXAMPLE XIV

25 A drop test apparatus comprising an injection nozzle inserted to within 1" of the bottom of a 1" x 8" test tube was employed to determine the ignition delay in milliseconds of N,N,N',N'-tetramethyl-1,2-diaminoethylene and N,N,N',N'-tetramethyl-1,2-propanediamine. 30 A small quantity of fuel (0.2 ml.) was placed in the bottom of the test tube and 0.3 ml. of white fuming nitric acid was injected into the fuel. A constant pressure nitrogen surge chamber provided a source of approximately 40 p.s.i.g. pressure to inject the oxidizer into the fuel. A solenoid coil actuated the injector to provide an accurately metered amount of oxidant. The ignition delay interval was determined as the time between contact of the oxidizer with the fuel and the presence of flame as sensed by a photocell. Table II gives the data obtained on the ignition delays obtained by this method.

Table II

| 45 | Material                                  | Ignition Delay with WFNA, Milliseconds at 75° F. | Ignition Delay with WFNA, Milliseconds at -40° F. |
|----|-------------------------------------------|--------------------------------------------------|---------------------------------------------------|
| 50 | N,N,N',N'-tetramethyl-1,2-diaminoethylene | 3.6                                              | 12.6                                              |
|    | N,N,N',N'-tetramethyl-1,2-propanediamine  | 16.9                                             | 13.3                                              |

<sup>1</sup> This value was obtained using a different acid and at a different time from the value given in Example XI.

55 As can be seen from the data given in the above Table II, the compound N,N,N',N'-tetramethyl-1,2-diaminoethylene, which is representative of the new compounds of my invention, exhibits an ignition delay which is superior to that of N,N,N',N'-tetramethyl-1,2-propanediamine, or any of the other hypergols tested in the other examples. These data show that my new hypergols are superior to any other hypergols previously known prior to my invention.

60 The superiority of my new compounds is further shown by a comparison with ethylene diamine, a known hypergolic fuel. Ethylene diamine has an ignition delay of 92.9 milliseconds at 75° F. as determined by the same apparatus and test procedure employed in Example XIV.

65 As will be evident to those skilled in the art, various modifications, substitutions and changes may be made or followed in the light of the foregoing disclosure without departing from the spirit or scope of this invention.

I claim:

1. A 1,2-diamino-1-alkene selected from the group consisting of N,N,N'N'-tetramethyl - 1,2 - diaminoethylene; N,N,N',N'-tetraethyl-1,2-diaminoethylene; and N,N'-dimethyl-N,N'-diethyl-1,2-diaminoethylene.
2. N,N,N',N'-tetramethyl-1,2-diaminoethylene.
3. N,N,N',N'-tetraethyl-1,2-diaminoethylene.
4. N,N' - dimethyl - N,N' - diethyl - 1,2 - diaminoethylene.

References Cited in the file of this patent

UNITED STATES PATENTS

|   |           |                       |                |
|---|-----------|-----------------------|----------------|
| 5 | 2,540,938 | Finch et al. -----    | Feb. 6, 1951   |
|   | 2,565,529 | Smith -----           | Aug. 28, 1951  |
|   | 2,617,827 | McKeever et al. ----- | Nov. 11, 1952  |
|   | 2,652,430 | Finch et al. -----    | Sept. 15, 1953 |
|   | 2,693,077 | Malina et al. -----   | Nov. 2, 1954   |
|   | 2,753,683 | Carmody -----         | July 10, 1956  |